



US010024000B2

(12) **United States Patent**  
**Barnholtz et al.**

(10) **Patent No.:** **US 10,024,000 B2**  
(45) **Date of Patent:** **\*Jul. 17, 2018**

(54) **FIBROUS STRUCTURES AND METHODS FOR MAKING SAME**

(75) Inventors: **Steven Lee Barnholtz**, West Chester, OH (US); **Paul Dennis Trokhan**, Hamilton, OH (US); **Michael Donald Suer**, Cincinnati, OH (US)

(73) Assignee: **The Procter & Gamble Company**, Cincinnati, OH (US)

(\*) Notice: Subject to any disclaimer, the term of this patent is extended or adjusted under 35 U.S.C. 154(b) by 1028 days.

This patent is subject to a terminal disclaimer.

(21) Appl. No.: **12/170,578**

(22) Filed: **Jul. 10, 2008**

(65) **Prior Publication Data**

US 2009/0084513 A1 Apr. 2, 2009

**Related U.S. Application Data**

(60) Provisional application No. 60/959,809, filed on Jul. 17, 2007.

(51) **Int. Cl.**

**D21H 27/30** (2006.01)  
**D04H 1/407** (2012.01)  
**D04H 1/425** (2012.01)  
**D04H 1/56** (2006.01)  
**D21H 11/12** (2006.01)  
**D21H 13/14** (2006.01)  
**D21H 15/06** (2006.01)  
**D21H 17/25** (2006.01)  
**D21H 17/28** (2006.01)

(52) **U.S. Cl.**

CPC ..... **D21H 27/30** (2013.01); **D04H 1/407** (2013.01); **D04H 1/425** (2013.01); **D04H 1/56** (2013.01); **D21H 11/12** (2013.01); **D21H**

13/14 (2013.01); **D21H 15/06** (2013.01); **D21H 17/25** (2013.01); **D21H 17/28** (2013.01)

(58) **Field of Classification Search**

CPC ..... D04H 13/002; D21H 11/12; D21H 13/14; D21H 15/06; D21H 17/25; D21H 17/28  
USPC .... 442/411, 413, 415, 416; 3/411, 413, 415, 3/416

See application file for complete search history.

(56)

**References Cited**

**U.S. PATENT DOCUMENTS**

2,175,045 A 10/1939 Vogel  
3,521,638 A 7/1970 Parrish  
3,838,692 A 10/1974 Levesque  
3,954,361 A 5/1976 Page  
4,100,324 A 7/1978 Anderson et al.

(Continued)

**FOREIGN PATENT DOCUMENTS**

DE 199 59 832 A1 7/2001  
EP 0 080 382 A1 11/1982

(Continued)

**OTHER PUBLICATIONS**

Complete Textile Glossary, Celanese Acetate (2001), definition for "filament".\*

(Continued)

*Primary Examiner* — Jeremy R Pierce

(74) *Attorney, Agent, or Firm* — C. Brant Cook

(57)

**ABSTRACT**

Fibrous structures that exhibit improved consumer recognizable properties, especially a VFS of greater than about 11 g/g, and to methods for making such fibrous structures are provided.

**11 Claims, 12 Drawing Sheets**



- |                              |                                         |
|------------------------------|-----------------------------------------|
| • Huggies (coform prior art) | • Huggies Wash Cloth (coform prior art) |
| ▲ Duramax                    | — Concert EBT.055/010 TBAL              |
| ■ LBAL-DUNI embossed         | • Bounty                                |
| ◆ Invention Example A        | ~ Invention Example B                   |

# US 10,024,000 B2

Page 2

| (56)                  | References Cited |                      |                   |         |                         |              |
|-----------------------|------------------|----------------------|-------------------|---------|-------------------------|--------------|
| U.S. PATENT DOCUMENTS |                  |                      |                   |         |                         |              |
| 4,118,531 A           | 10/1978          | Hauser               | 6,621,679 B1      | 9/2003  | Segervall               |              |
| 4,139,699 A           | 2/1979           | Hernandez et al.     | 6,686,303 B1      | 2/2004  | Haynes et al.           |              |
| 4,203,939 A           | 5/1980           | Drachenberg et al.   | 6,709,526 B1      | 3/2004  | Bailey et al.           |              |
| 4,243,480 A           | 1/1981           | Hernandez et al.     | 6,739,023 B2      | 5/2004  | Vonfeldt et al.         |              |
| 4,295,987 A *         | 10/1981          | Parks .....          | 6,759,356 B1      | 7/2004  | Myers                   |              |
| 4,355,066 A           | 10/1982          | Newman               | 6,797,226 B2      | 9/2004  | Annable                 |              |
| 4,370,289 A           | 1/1983           | Sorenson             | 6,811,638 B2      | 11/2004 | Close et al.            |              |
| 4,436,780 A           | 3/1984           | Hotchkiss et al.     | 6,823,568 B1      | 11/2004 | Kobayashi et al.        |              |
| 4,604,313 A           | 8/1986           | McFarland et al.     | 6,836,937 B1      | 1/2005  | Boscolo                 |              |
| 4,623,576 A           | 11/1986          | Lloyd et al.         | 6,946,413 B2      | 9/2005  | Lange et al.            |              |
| 4,634,621 A           | 1/1987           | Manning et al.       | 6,979,386 B1      | 12/2005 | Wallajapet et al.       |              |
| 4,636,418 A           | 1/1987           | Kennard et al.       | 6,986,932 B2      | 1/2006  | Zink et al.             |              |
| 4,675,226 A           | 6/1987           | Ott                  | 6,992,028 B2      | 1/2006  | Thomaschefskey et al.   |              |
| 4,720,415 A           | 1/1988           | Vander Wielen et al. | 7,029,620 B2      | 1/2006  | Gordon et al.           |              |
| 4,724,114 A           | 2/1988           | McFarland et al.     | 7,000,000 B1      | 2/2006  | O'Brien                 |              |
| 4,786,550 A           | 11/1988          | McFarland et al.     | 7,028,429 B1      | 4/2006  | Vinson et al.           |              |
| 4,803,117 A           | 2/1989           | Daponte              | 7,041,369 B1      | 5/2006  | Mackey et al.           |              |
| 4,851,168 A           | 7/1989           | Graiver et al.       | 7,176,150 B2      | 2/2007  | Kopacz et al.           |              |
| 4,855,179 A           | 8/1989           | Bourland et al.      | 7,410,683 B2      | 8/2008  | Curro et al.            |              |
| 4,863,779 A           | 9/1989           | Daponte              | 7,425,517 B2      | 9/2008  | Deka et al.             |              |
| 4,879,170 A           | 11/1989          | Radwanski et al.     | 7,696,109 B2      | 4/2010  | Ouellette et al.        |              |
| 4,885,202 A           | 12/1989          | Lloyd et al.         | 7,879,172 B2      | 2/2011  | Kopcz et al.            |              |
| 4,906,513 A           | 3/1990           | Kebbell et al.       | 7,902,096 B2      | 3/2011  | Brandner et al.         |              |
| 4,931,355 A           | 6/1990           | Radwanski et al.     | 7,994,079 B2      | 8/2011  | Chen et al.             |              |
| 4,939,016 A           | 7/1990           | Radwanski et al.     | 7,994,081 B2      | 8/2011  | Farrell et al.          |              |
| 4,970,104 A           | 11/1990          | Radwanski            | 7,998,889 B2      | 8/2011  | Stralin et al.          |              |
| 5,087,506 A           | 2/1992           | Palumbo              | 8,017,534 B2      | 9/2011  | Harvey et al.           |              |
| 5,120,888 A           | 6/1992           | Nohr et al.          | 2003/0024662 A1 * | 2/2003  | Besemer et al. .....    | 162/9        |
| 5,145,727 A           | 9/1992           | Potts et al.         | 2003/0073367 A1   | 4/2003  | Kopacz et al.           |              |
| 5,149,576 A           | 9/1992           | Potts et al.         | 2003/0105650 A1 * | 6/2003  | Griesbach et al. .....  | 128/849      |
| 5,204,165 A           | 4/1993           | Schortmann           | 2003/0116890 A1 * | 6/2003  | Chambers et al. .....   | 264/518      |
| 5,227,107 A           | 7/1993           | Dickenson et al.     | 2003/0220039 A1   | 7/2003  | Krautkramer et al.      |              |
| 5,254,133 A           | 10/1993          | Seid                 | 2004/0048542 A1   | 7/2003  | Whitmore et al.         |              |
| 5,254,399 A           | 10/1993          | Oku et al.           | 2004/0065422 A1   | 8/2003  | Krautkramer et al.      |              |
| 5,284,703 A           | 2/1994           | Everhart et al.      | 2004/0087237 A1   | 10/2003 | Keck et al.             |              |
| 5,350,624 A           | 9/1994           | Georger et al.       | 2004/0096656 A1   | 11/2003 | Chen et al.             |              |
| 5,409,768 A           | 4/1995           | Dickenson et al.     | 2004/0106723 A1   | 3/2004  | Thomaschefskey et al.   |              |
| 5,427,696 A           | 6/1995           | Phan et al.          | 2004/0116018 A1 * | 4/2004  | Hu et al.               |              |
| 5,436,066 A           | 7/1995           | Chen                 | 2004/0163781 A1   | 5/2004  | Garnier et al.          |              |
| 5,476,616 A           | 12/1995          | Schwarz              | 2004/0181199 A1   | 6/2004  | Bond                    |              |
| 5,508,102 A           | 4/1996           | Georger et al.       | 2005/0020170 A1   | 7/2005  | Fenwick .....           | A61F 13/8405 |
| 5,509,915 A           | 4/1996           | Hanson et al.        | 2005/0056956 A1   | 8/2005  | 442/164                 |              |
| 5,536,563 A           | 7/1996           | Shah et al.          | 2005/0090175 A1   | 9/2004  | Hernandez-Munoa et al.  |              |
| 5,539,056 A           | 7/1996           | Yang et al.          | 2005/0103455 A1   | 10/2004 | Moberg-Alehammar et al. |              |
| 5,587,225 A           | 12/1996          | Griesbach et al.     | 2005/0112980 A1   | 11/2004 | Stralin et al.          |              |
| 5,597,873 A           | 1/1997           | Chambers et al.      | 2005/0130536 A1   | 12/2004 | Bergholm et al.         |              |
| 5,611,890 A           | 3/1997           | Vinson et al.        | 2005/0130544 A1   | 1/2005  | Edwards et al.          |              |
| 5,629,080 A           | 5/1997           | Gupta et al.         | 2005/0133177 A1   | 3/2005  | Strandqvist et al.      |              |
| 5,652,048 A           | 7/1997           | Haynes et al.        | 2005/0136765 A1   | 6/2005  | Siebers et al.          |              |
| 5,811,178 A           | 9/1998           | Adam et al.          | 2005/0136772 A1   | 6/2005  | Cheng et al.            |              |
| 5,814,570 A           | 9/1998           | Cohen                | 2005/0136778 A1   | 7/2005  | Stralin et al.          |              |
| 5,853,867 A           | 12/1998          | Harada et al.        | 2005/0137540 A1   | 8/2005  | Berba et al.            |              |
| 5,948,710 A           | 9/1999           | Pomplun et al.       | 2005/0148264 A1   | 9/2005  | Chmielewski et al.      |              |
| 5,952,251 A           | 9/1999           | Jackson et al.       | 2005/0159065 A1   | 10/2005 | Forry et al.            |              |
| 6,103,061 A           | 8/2000           | Anderson et al.      | 2005/0177122 A1   | 11/2005 | Varona et al.           |              |
| 6,150,005 A           | 11/2000          | Williams et al.      | 2005/0245159 A1   | 12/2005 | Shannon et al.          |              |
| 6,172,276 B1          | 1/2001           | Hetzler et al.       | 2005/0247416 A1   | 1/2006  | Kleinsmith              |              |
| 6,177,370 B1          | 1/2001           | Skoog et al.         | 2005/0274470 A1   | 2/2006  | Manifold et al.         |              |
| 6,200,120 B1          | 3/2001           | Fish et al.          | 2006/0086633 A1   | 3/2006  | Shaffer et al.          |              |
| 6,296,936 B1          | 10/2001          | Yahiaoui et al.      | 2006/0088697 A1   | 4/2006  | Cabell et al.           |              |
| 6,319,342 B1          | 11/2001          | Riddell              | 2007/0010153 A1   | 5/2006  | Dunbar et al.           |              |
| 6,348,133 B1          | 2/2002           | Woodrum              | 2007/0039704 A1   | 6/2006  | Dunbar et al.           |              |
| 6,348,253 B1          | 2/2002           | Daley et al.         | 2007/0049153 A1   | 7/2006  | Neveu                   |              |
| 6,361,784 B1          | 3/2002           | Brennan et al.       | 2007/0063091 A1   | 8/2006  | Zoch et al.             |              |
| 6,383,336 B1          | 5/2002           | Shannon              | 2007/0077841 A1   | 9/2006  | Ouellette et al.        |              |
| 6,417,120 B1          | 7/2002           | Mitchler et al.      | 2007/0202766 A1   | 10/2006 | Polat et al.            |              |
| 6,423,884 B1          | 7/2002           | Oehmen               | 2007/0232180 A1   | 11/2006 | Vinson .....            | A47K 10/16   |
| 6,465,073 B1          | 10/2002          | Morman et al.        | 2007/0269627 A1 * | 12/2006 | 428/43                  |              |
| 6,488,801 B1          | 12/2002          | Bodaghi et al.       |                   |         |                         |              |
| 6,494,974 B2          | 12/2002          | Riddell              |                   |         |                         |              |
| 6,503,370 B2          | 1/2003           | Hollmark et al.      | 2007/0272381 A1   | 1/2007  | Elony et al.            |              |
| 6,506,873 B1          | 1/2003           | Ryan et al.          | 2008/000602 A1    | 2/2007  | Dyer et al.             |              |
| 6,550,115 B1          | 4/2003           | Skoog et al.         | 2008/008853 A1    | 3/2007  | Hupp et al.             |              |
| 6,589,892 B1          | 7/2003           | Smith et al.         | 2008/0041543 A1   | 4/2007  | Dyer et al.             |              |
| 6,608,236 B1          | 8/2003           | Burns et al.         | 2008/0050996 A1   | 5/2007  | Stralin et al.          |              |

| (56)                                                                                                                                                                                                                                                                                                                               | References Cited |                  |    |                   |         |  |
|------------------------------------------------------------------------------------------------------------------------------------------------------------------------------------------------------------------------------------------------------------------------------------------------------------------------------------|------------------|------------------|----|-------------------|---------|--|
| U.S. PATENT DOCUMENTS                                                                                                                                                                                                                                                                                                              |                  |                  |    |                   |         |  |
| 2008/0142178 A1                                                                                                                                                                                                                                                                                                                    | 6/2008           | Haubrich et al.  | WO | WO 02/50357 A1    | 6/2002  |  |
| 2008/0241538 A1                                                                                                                                                                                                                                                                                                                    | 10/2008          | Lee et al.       | WO | WO 02/053003 A2   | 7/2002  |  |
| 2008/0248239 A1                                                                                                                                                                                                                                                                                                                    | 10/2008          | Pomeroy et al.   | WO | WO 02/053365 A2   | 7/2002  |  |
| 2009/0022960 A1                                                                                                                                                                                                                                                                                                                    | 1/2009           | Suer et al.      | WO | WO 03/050347 A1   | 6/2003  |  |
| 2009/0022983 A1                                                                                                                                                                                                                                                                                                                    | 1/2009           | Cabell et al.    | WO | WO 03/080905 A1   | 10/2003 |  |
| 2009/0023839 A1                                                                                                                                                                                                                                                                                                                    | 1/2009           | Barnholtz et al. | WO | WO 2004/092474 A2 | 10/2004 |  |
| 2009/0151748 A1                                                                                                                                                                                                                                                                                                                    | 6/2009           | Ridenhour        | WO | WO 2005/065516 A2 | 7/2005  |  |
| 2009/0220741 A1                                                                                                                                                                                                                                                                                                                    | 9/2009           | Manifold et al.  | WO | WO 2005/065932    | 7/2005  |  |
| 2009/0220769 A1                                                                                                                                                                                                                                                                                                                    | 9/2009           | Manifold et al.  | WO | WO 2005/073446 A1 | 8/2005  |  |
| 2010/0239825 A1                                                                                                                                                                                                                                                                                                                    | 9/2010           | Sheehan et al.   | WO | WO 2005/080497 A1 | 9/2005  |  |
| 2010/0326612 A1                                                                                                                                                                                                                                                                                                                    | 12/2010          | Hupp et al.      | WO | WO 2005/106085 A1 | 11/2005 |  |
| 2011/0100574 A1                                                                                                                                                                                                                                                                                                                    | 5/2011           | Barnholtz et al. | WO | WO 2005/118934 A1 | 12/2005 |  |
| 2011/0104419 A1                                                                                                                                                                                                                                                                                                                    | 5/2011           | Barnholtz et al. | WO | WO 2006/027810 A1 | 3/2006  |  |
| 2011/0104444 A1                                                                                                                                                                                                                                                                                                                    | 5/2011           | Barnholtz et al. | WO | WO 2006/060816 A1 | 6/2006  |  |
| 2011/0104493 A1                                                                                                                                                                                                                                                                                                                    | 5/2011           | Barnholtz et al. | WO | WO 2006/069120 A2 | 6/2006  |  |
| 2011/0104970 A1                                                                                                                                                                                                                                                                                                                    | 5/2011           | Barnholtz et al. | WO | WO 2007/070064 A1 | 6/2007  |  |
| 2011/0209840 A1                                                                                                                                                                                                                                                                                                                    | 9/2011           | Barnholtz et al. | WO | WO 2007/070075 A1 | 6/2007  |  |
| 2011/0220310 A1                                                                                                                                                                                                                                                                                                                    | 9/2011           | Polat et al.     | WO | WO 2007/078344 A1 | 7/2007  |  |
| 2011/0244199 A1                                                                                                                                                                                                                                                                                                                    | 10/2011          | Brennan et al.   | WO | WO 2007/092303 A2 | 8/2007  |  |
| FOREIGN PATENT DOCUMENTS                                                                                                                                                                                                                                                                                                           |                  |                  |    |                   |         |  |
| EP 0 156 649 A2                                                                                                                                                                                                                                                                                                                    | 10/1985          |                  | WO | WO 2007/098449 A1 | 8/2007  |  |
| EP 1 156 160 A2                                                                                                                                                                                                                                                                                                                    | 10/1985          |                  | WO | WO 2007/100936 A2 | 9/2007  |  |
| EP 0 294 137 A1                                                                                                                                                                                                                                                                                                                    | 12/1988          |                  | WO | WO 2007/124866 A1 | 11/2007 |  |
| EP 0 308 320 A2                                                                                                                                                                                                                                                                                                                    | 3/1989           |                  | WO | WO 2007/135624 A2 | 11/2007 |  |
| EP 0 333 209 B1                                                                                                                                                                                                                                                                                                                    | 9/1989           |                  | WO | WO 2008/005500 A2 | 1/2008  |  |
| EP 0 341 977 A2                                                                                                                                                                                                                                                                                                                    | 11/1989          |                  | WO | WO 2008/050311 A2 | 5/2008  |  |
| EP 0423 619 A1                                                                                                                                                                                                                                                                                                                     | 4/1991           |                  | WO | WO 2008/073101 A1 | 6/2008  |  |
| EP 0 205 242 B2                                                                                                                                                                                                                                                                                                                    | 12/1991          |                  | WO | WO 2009/010938 A1 | 1/2009  |  |
| EP 0 357 496 BI                                                                                                                                                                                                                                                                                                                    | 5/1994           |                  | WO | WO 2009/010939 A2 | 1/2009  |  |
| EP 0 865 755 A1                                                                                                                                                                                                                                                                                                                    | 9/1998           |                  | WO | WO 2009/010940 A2 | 1/2009  |  |
| EP 0 590 307 B1                                                                                                                                                                                                                                                                                                                    | 12/1998          |                  | WO | WO 2009/010941 A2 | 1/2009  |  |
| EP 0 992 338 A2                                                                                                                                                                                                                                                                                                                    | 4/2000           |                  | WO | WO 2009/010942 A2 | 1/2009  |  |
| EP 1 132 427 A1                                                                                                                                                                                                                                                                                                                    | 9/2001           |                  | WO | WO 2006/060813 A1 | 6/2009  |  |
| EP 1 156 147 A1                                                                                                                                                                                                                                                                                                                    | 11/2001          |                  | WO | WO 2006/060815 A2 | 6/2009  |  |
| EP 1 300 511 A2                                                                                                                                                                                                                                                                                                                    | 4/2003           |                  | WO | WO 2009/105490 A1 | 8/2009  |  |
| EP 1 589 137 A1                                                                                                                                                                                                                                                                                                                    | 10/2005          |                  | WO | WO 2011/019908 A1 | 2/2011  |  |
| EP 1 887 036 A2                                                                                                                                                                                                                                                                                                                    | 2/2008           |                  | WO | WO 2011/053677 A1 | 5/2011  |  |
| EP 1 504 145 B1                                                                                                                                                                                                                                                                                                                    | 11/2008          |                  |    |                   |         |  |
| EP 2 028 296 A1                                                                                                                                                                                                                                                                                                                    | 2/2009           |                  |    |                   |         |  |
| GB 2113731 A                                                                                                                                                                                                                                                                                                                       | 8/1983           |                  |    |                   |         |  |
| JP 59-211667 A                                                                                                                                                                                                                                                                                                                     | 11/1984          |                  |    |                   |         |  |
| JP 08-174735 A                                                                                                                                                                                                                                                                                                                     | 7/1996           |                  |    |                   |         |  |
| JP 2000/303335 A2                                                                                                                                                                                                                                                                                                                  | 10/2000          |                  |    |                   |         |  |
| JP 2002/088660 A                                                                                                                                                                                                                                                                                                                   | 3/2002           |                  |    |                   |         |  |
| JP 2004-141255 A                                                                                                                                                                                                                                                                                                                   | 5/2004           |                  |    |                   |         |  |
| JP 2005/218525 A2                                                                                                                                                                                                                                                                                                                  | 8/2005           |                  |    |                   |         |  |
| WO WO 92/07985 A1                                                                                                                                                                                                                                                                                                                  | 5/1992           |                  |    |                   |         |  |
| WO WO 94/19179 A1                                                                                                                                                                                                                                                                                                                  | 9/1994           |                  |    |                   |         |  |
| WO WO 97/37757 A1                                                                                                                                                                                                                                                                                                                  | 10/1997          |                  |    |                   |         |  |
| WO WO 98/03713 A1                                                                                                                                                                                                                                                                                                                  | 1/1998           |                  |    |                   |         |  |
| WO WO 98/27257 A2                                                                                                                                                                                                                                                                                                                  | 6/1998           |                  |    |                   |         |  |
| WO WO 98/36117 A1                                                                                                                                                                                                                                                                                                                  | 8/1998           |                  |    |                   |         |  |
| WO WO 98/55295 A1                                                                                                                                                                                                                                                                                                                  | 12/1998          |                  |    |                   |         |  |
| WO WO 00/11998 A1                                                                                                                                                                                                                                                                                                                  | 3/2000           |                  |    |                   |         |  |
| WO WO 00/21476 A1                                                                                                                                                                                                                                                                                                                  | 4/2000           |                  |    |                   |         |  |
| WO WO 00/29655 A1                                                                                                                                                                                                                                                                                                                  | 5/2000           |                  |    |                   |         |  |
| WO WO 00/38565 A1                                                                                                                                                                                                                                                                                                                  | 7/2000           |                  |    |                   |         |  |
| WO WO 00/63486 A1                                                                                                                                                                                                                                                                                                                  | 10/2000          |                  |    |                   |         |  |
| WO WO 01/09023 A1                                                                                                                                                                                                                                                                                                                  | 2/2001           |                  |    |                   |         |  |
| WO WO 01/66345 A1                                                                                                                                                                                                                                                                                                                  | 9/2001           |                  |    |                   |         |  |
| OTHER PUBLICATIONS                                                                                                                                                                                                                                                                                                                 |                  |                  |    |                   |         |  |
| International Search Report, dated Dec. 17, 2008.                                                                                                                                                                                                                                                                                  |                  |                  |    |                   |         |  |
| Anonymous, "NanoDispense® Contact Angle Measurements", <i>First Ten Angstroms</i> , (Oct. 3, 2004). Retrieved from the Internet: URL: <a href="http://www.firstenangstroms.com/pdfdocs/NanoDispenseExamples.pdf">http://www.firstenangstroms.com/pdfdocs/NanoDispenseExamples.pdf</a> , (retrieved Feb. 15, 2011) Entire document. |                  |                  |    |                   |         |  |
| Meyer, et al., "Comparison between different presentations of pore size distribution in porous materials." <i>Fresenius J. Anal. Chem.</i> 1999. 363: pp. 174-178.                                                                                                                                                                 |                  |                  |    |                   |         |  |
| Office Action U.S. Appl. No. 12/170,585 dated Aug. 20, 2010.                                                                                                                                                                                                                                                                       |                  |                  |    |                   |         |  |
| Final Office Action U.S. Appl. No. 12/170,585 dated Jan. 31, 2011.                                                                                                                                                                                                                                                                 |                  |                  |    |                   |         |  |
| Office Action U.S. Appl. No. 12/170,575 dated May 29, 2010.                                                                                                                                                                                                                                                                        |                  |                  |    |                   |         |  |
| Office Action U.S. Appl. No. 12/170,575 dated Oct. 1, 2009.                                                                                                                                                                                                                                                                        |                  |                  |    |                   |         |  |
| Final Office Action U.S. Appl. No. 12/170,575 dated Mar. 11, 2010.                                                                                                                                                                                                                                                                 |                  |                  |    |                   |         |  |
| Office Action U.S. Appl. No. 12/170,557 dated Dec. 29, 2010.                                                                                                                                                                                                                                                                       |                  |                  |    |                   |         |  |
| Final Office Action U.S. Appl. No. 12/170,557 dated Apr. 18, 2011.                                                                                                                                                                                                                                                                 |                  |                  |    |                   |         |  |
| Office Action U.S. Appl. No. 12/170,565 dated Mar. 2, 2011.                                                                                                                                                                                                                                                                        |                  |                  |    |                   |         |  |
| All Office Actions in U.S. Appl. Nos. 13/106,302, 12/170,578, 12/170,575, 12/170,557, 12/917,535, 12/917,547, 12/917,558, 12/917,574, 12/917,585, and 13/076,492.                                                                                                                                                                  |                  |                  |    |                   |         |  |
| All Office Actions in U.S. Appl. Nos. 13/106,302, 12/170,578, 12/170,575, 14/475,699, 12/170,557, 12/917,535, 12/917,547, 12/917,558, 12/917,574, 12/917,585, and 13/076,492.                                                                                                                                                      |                  |                  |    |                   |         |  |
| U.S. Appl. No. 14/475,699, filed Sep. 3, 2014, Barnholtz, et al.                                                                                                                                                                                                                                                                   |                  |                  |    |                   |         |  |

\* cited by examiner



Fig. 1



Fig. 2



Fig. 3



Fig. 4



Fig. 5



Fig. 6



Fig. 7



Fig. 8



Fig. 9



Fig. 10



Fig. 11



Fig. 12



Fig. 13



Fig. 14



Fig. 16A



Fig. 16



Fig. 17A



Fig. 17

## 1

FIBROUS STRUCTURES AND METHODS  
FOR MAKING SAMECROSS REFERENCE TO RELATED  
APPLICATIONS

This application claims the benefit of U.S. Provisional Application No. 60/959,809, filed Jul. 17, 2007.

## FIELD OF THE INVENTION

The present invention relates to fibrous structures and more particularly to fibrous structures that exhibit improved consumer recognizable properties, especially a VFS of greater than about 11 g/g, and to methods for making such fibrous structures.

## BACKGROUND OF THE INVENTION

Consumers of fibrous structures, especially paper towels, require absorbency (such as absorption capacity and/or rate of absorption) and strength properties in their fibrous structures. To date, no known fibrous structures provide consumers optimal absorbency and strength properties.

The problem faced by formulators is how to produce fibrous structures that exhibit improved absorbency and strength properties to meet the consumers' needs.

Accordingly, there is a need for fibrous structures that exhibit improved absorbency and/or strength properties that meet consumers' needs compared to known fibrous structures and for methods for making such fibrous structures.

## SUMMARY OF THE INVENTION

The present invention solves the problem identified above by fulfilling the needs of the consumers by providing fibrous structures that exhibit improved absorbency and/or strength properties and methods for making such fibrous structures.

In one example of the present invention, a fibrous structure that exhibits a VFS of greater than about 11 g/g as measured by the VFS Test Method described herein is provided.

In another example of the present invention, a fibrous structure that exhibits a pore volume distribution such that less than about 20% of the total pore volume present in the fibrous structure exists in pores of radii of from about 1  $\mu\text{m}$  to about 50  $\mu\text{m}$  as measured by the Pore Volume Distribution Test Method described herein, wherein the fibrous structure exhibits a VFS of greater than about 11 g/g as measured by the VFS Test Method described herein is provided.

In still another example of the present invention, an osmotic material-free fibrous structure that exhibits a VFS of greater than about 11 g/g as measured by the VFS Test Method described herein is provided.

In still another example of the present invention, a fibrous structure that exhibits a VFS of greater than about 11 g/g and one or more of the following: a Dry CD Tensile Modulus of less than about 1500 g/cm and/or a Wet CD TEA of greater than about 35 (g·in)/in<sup>2</sup> and/or a Wet MD TEA of greater than about 40 (g·in)/in<sup>2</sup> is provided.

In another example of the present invention, a fibrous structure that exhibits one or more of the following properties:

- a. a Dry CD Tensile Modulus of less than about 1500 g/cm;
- b. a Wet CD TEA of greater than about 35 (g·in)/in<sup>2</sup>
- c. a Wet MD TEA of greater than about 40 (g·in)/in<sup>2</sup>; and
- d. mixtures thereof, is provided.

In even still another example of the present invention, a method for making a fibrous structure according to the present invention, the method comprising the step of com-

## 2

bining a plurality of filaments to form a fibrous structure that exhibits improved absorbency and/or strength properties is provided.

The present invention solves the problem identified above by fulfilling the needs of the consumers by providing fibrous structures that exhibit a novel pore volume distribution and methods for making such fibrous structures.

In yet another example of the present invention, a sanitary tissue product comprising a fibrous structure according to the present invention is provided.

Accordingly, the present invention provides fibrous structures that solve the problems described above by providing fibrous structures that exhibit improved absorbency and/or strength properties compared to known fibrous structures and to methods for making such fibrous structures.

## BRIEF DESCRIPTION OF THE DRAWINGS

FIG. 1 is a Pore Volume Distribution graph of various fibrous structures, including a fibrous structure according to the present invention, showing the Ending Pore Radius of from 1  $\mu\text{m}$  to 1000  $\mu\text{m}$  and the Capacity of Water in Pores;

FIG. 2 is a Pore Volume Distribution graph of various fibrous structures, including a fibrous structure according to the present invention, showing the Ending Pore Radius of from 1  $\mu\text{m}$  to 300  $\mu\text{m}$  and the Capacity of Water in Pores;

FIG. 3 is a schematic representation of an example of a fibrous structure according to the present invention;

FIG. 4 is a schematic, cross-sectional representation of FIG. 3 taken along line 4-4;

FIG. 5 is a schematic representation of another example of a fibrous structure according to the present invention;

FIG. 6 is a schematic, cross-sectional representation of another example of a fibrous structure according to the present invention;

FIG. 7 is a schematic, cross-sectional representation of another example of a fibrous structure according to the present invention;

FIG. 8 is a schematic representation of another example of a fibrous structure in roll form according to the present invention;

FIG. 9 is a schematic representation of another example of a fibrous structure;

FIG. 10 is a schematic representation of an example of a process for making a fibrous structure according to the present invention;

FIG. 11 is a schematic representation of an example of a filament-forming hole and fluid-releasing hole from a suitable die useful in making a fibrous structure according to the present invention;

FIG. 12 is a scanning electronmicrograph of a fibrous structure made by a known die;

FIG. 13 is a scanning electronmicrograph of a fibrous structure made by a die according to the present invention;

FIG. 14 is a schematic representation of an example of a solid additive spreader useful in the processes of the present invention;

FIG. 15 is a schematic representation of another example of a solid additive spreader useful in the processes of the present invention;

FIG. 16 is a diagram of a support rack utilized in the HFS and VFS Test Methods described herein;

FIG. 17 is a diagram of a support rack cover utilized in the HFS and VFS Test Methods described herein.

DETAILED DESCRIPTION OF THE  
INVENTION

## 65 Definitions

“Fibrous structure” as used herein means a structure that comprises one or more filaments and/or fibers. In one

example, a fibrous structure according to the present invention means an orderly arrangement of filaments and/or fibers within a structure in order to perform a function. Nonlimiting examples of fibrous structures of the present invention include paper, fabrics (including woven, knitted, and non-woven), and absorbent pads (for example for diapers or feminine hygiene products).

Nonlimiting examples of processes for making fibrous structures include known wet-laid papermaking processes and air-laid papermaking processes. Such processes typically include steps of preparing a fiber composition in the form of a suspension in a medium, either wet, more specifically aqueous medium, or dry, more specifically gaseous, i.e. with air as medium. The aqueous medium used for wet-laid processes is oftentimes referred to as a fiber slurry. The fibrous slurry is then used to deposit a plurality of fibers onto a forming wire or belt such that an embryonic fibrous structure is formed, after which drying and/or bonding the fibers together results in a fibrous structure. Further processing the fibrous structure may be carried out such that a finished fibrous structure is formed. For example, in typical papermaking processes, the finished fibrous structure is the fibrous structure that is wound on the reel at the end of papermaking, and may subsequently be converted into a finished product, e.g. a sanitary tissue product.

The fibrous structures of the present invention may be homogeneous or may be layered. If layered, the fibrous structures may comprise at least two and/or at least three and/or at least four and/or at least five layers.

The fibrous structures of the present invention may comprise tufts or may be non-tufted.

The fibrous structures of the present invention may be co-formed fibrous structures.

“Co-formed fibrous structure” as used herein means that the fibrous structure comprises a mixture of at least two different materials wherein at least one of the materials comprises a filament, such as a polypropylene filament, and at least one other material, different from the first material, comprises a solid additive, such as a fiber and/or a particulate. In one example, a co-formed fibrous structure comprises solid additives, such as fibers, such as wood pulp fibers, and filaments, such as polypropylene filaments.

“Osmotic material” as used herein is a material that absorbs liquids by transfer of the liquids across the periphery of the material, forming a gelatinous substance, which imbibes the liquids and tightly holds the liquids. In one example, osmotic materials retain greater than 5 times their weight of deionized water when subjected to centrifugal forces of less than or equal to 3000 G’s for 10 to 15 minutes. In comparison, typical capillary absorbents retain about 1 times their weight under similar conditions. Nonlimiting examples of osmotic materials include crosslinked polyacrylic acids and/or crosslinked carboxymethylcellulose.

“Osmotic material-free” as used herein with respect to a fibrous structure means that the fibrous structure contains less than an amount of osmotic material that results in the fibrous structure exhibiting a VFS of greater than about 11 g/g as measured by the VFS Test Method described herein. In one example, an osmotic material-free fibrous structure comprises 0% by dry weight of the fibrous structure of osmotic material.

“Solid additive” as used herein means a fiber and/or a particulate.

“Particulate” as used herein means a granular substance or powder.

“Fiber” and/or “Filament” as used herein means an elongate particulate having an apparent length greatly exceeding

its apparent width, i.e. a length to diameter ratio of at least about 10. For purposes of the present invention, a “fiber” is an elongate particulate as described above that exhibits a length of less than 5.08 cm (2 in.) and a “filament” is an elongate particulate as described above that exhibits a length of greater than or equal to 5.08 cm (2 in.).

Fibers are typically considered discontinuous in nature. Nonlimiting examples of fibers include wood pulp fibers and synthetic staple fibers such as polyester fibers.

10 Filaments are typically considered continuous or substantially continuous in nature. Filaments are relatively longer than fibers. Nonlimiting examples of filaments include melt-blown and/or spunbond filaments. Nonlimiting examples of materials that can be spun into filaments include natural polymers, such as starch, starch derivatives, cellulose and cellulose derivatives, hemicellulose, hemicellulose derivatives, and synthetic polymers including, but not limited to polyvinyl alcohol filaments and/or polyvinyl alcohol derivative filaments, and thermoplastic polymer filaments, such as 15 polyesters, nylons, polyolefins such as polypropylene filaments, polyethylene filaments, and biodegradable or compostable thermoplastic fibers such as polylactic acid filaments, polyhydroxyalkanoate filaments and polycaprolactone filaments. The filaments may be monocomponent or multicomponent, such as bicomponent filaments.

In one example of the present invention, “fiber” refers to papermaking fibers. Papermaking fibers useful in the present invention include cellulosic fibers commonly known as 30 wood pulp fibers. Applicable wood pulps include chemical pulps, such as Kraft, sulfite, and sulfate pulps, as well as mechanical pulps including, for example, groundwood, thermomechanical pulp and chemically modified thermomechanical pulp. Chemical pulps, however, may be preferred 35 since they impart a superior tactile sense of softness to tissue sheets made therefrom. Pulps derived from both deciduous trees (hereinafter, also referred to as “hardwood”) and coniferous trees (hereinafter, also referred to as “softwood”) may be utilized. The hardwood and softwood fibers can be 40 blended, or alternatively, can be deposited in layers to provide a stratified web. U.S. Pat. Nos. 4,300,981 and 3,994,771 are incorporated herein by reference for the purpose of disclosing layering of hardwood and softwood fibers. Also applicable to the present invention are fibers 45 derived from recycled paper, which may contain any or all of the above categories as well as other non-fibrous materials such as fillers and adhesives used to facilitate the original papermaking.

In addition to the various wood pulp fibers, other cellulosic fibers such as cotton linters, rayon, lyocell and bagasse can be used in this invention. Other sources of cellulose in the form of fibers or capable of being spun into fibers include grasses and grain sources.

“Sanitary tissue product” as used herein means a soft, low 55 density (i.e. <about 0.15 g/cm<sup>3</sup>) web useful as a wiping implement for post-urinary and post-bowel movement cleaning (toilet tissue), for otorhinolaryngological discharges (facial tissue), and multi-functional absorbent and cleaning uses (absorbent towels). The sanitary tissue product may be convolutedly wound upon itself about a core or without a core to form a sanitary tissue product roll.

In one example, the sanitary tissue product of the present invention comprises a fibrous structure according to the present invention.

60 65 The sanitary tissue products of the present invention may exhibit a basis weight between about 10 g/m<sup>2</sup> to about 120 g/m<sup>2</sup> and/or from about 15 g/m<sup>2</sup> to about 110 g/m<sup>2</sup> and/or

from about 20 g/m<sup>2</sup> to about 100 g/m<sup>2</sup> and/or from about 30 to 90 g/m<sup>2</sup>. In addition, the sanitary tissue product of the present invention may exhibit a basis weight between about 40 g/m<sup>2</sup> to about 120 g/m<sup>2</sup> and/or from about 50 g/m<sup>2</sup> to about 110 g/m<sup>2</sup> and/or from about 55 g/m<sup>2</sup> to about 105 g/m<sup>2</sup> and/or from about 60 to 100 g/m<sup>2</sup>.

The sanitary tissue products of the present invention may exhibit a total dry tensile strength of greater than about 59 g/cm (150 g/in) and/or from about 78 g/cm (200 g/in) to about 394 g/cm (1000 g/in) and/or from about 98 g/cm (250 g/in) to about 335 g/cm (850 g/in). In addition, the sanitary tissue product of the present invention may exhibit a total dry tensile strength of greater than about 196 g/cm (500 g/in) and/or from about 196 g/cm (500 g/in) to about 394 g/cm (1000 g/in) and/or from about 216 g/cm (550 g/in) to about 335 g/cm (850 g/in) and/or from about 236 g/cm (600 g/in) to about 315 g/cm (800 g/in). In one example, the sanitary tissue product exhibits a total dry tensile strength of less than about 394 g/cm (1000 g/in) and/or less than about 335 g/cm (850 g/in).

In another example, the sanitary tissue products of the present invention may exhibit a total dry tensile strength of greater than about 196 g/cm (500 g/in) and/or greater than about 236 g/cm (600 g/in) and/or greater than about 276 g/cm (700 g/in) and/or greater than about 315 g/cm (800 g/in) and/or greater than about 354 g/cm (900 g/in) and/or greater than about 394 g/cm (1000 g/in) and/or from about 315 g/cm (800 g/in) to about 1968 g/cm (5000 g/in) and/or from about 354 g/cm (900 g/in) to about 1181 g/cm (3000 g/in) and/or from about 354 g/cm (900 g/in) to about 984 g/cm (2500 g/in) and/or from about 394 g/cm (1000 g/in) to about 787 g/cm (2000 g/in).

The sanitary tissue products of the present invention may exhibit an initial total wet tensile strength of less than about 78 g/cm (200 g/in) and/or less than about 59 g/cm (150 g/in) and/or less than about 39 g/cm (100 g/in) and/or less than about 29 g/cm (75 g/in).

The sanitary tissue products of the present invention may exhibit an initial total wet tensile strength of greater than about 118 g/cm (300 g/in) and/or greater than about 157 g/cm (400 g/in) and/or greater than about 196 g/cm (500 g/in) and/or greater than about 236 g/cm (600 g/in) and/or greater than about 276 g/cm (700 g/in) and/or greater than about 315 g/cm (800 g/in) and/or greater than about 354 g/cm (900 g/in) and/or greater than about 394 g/cm (1000 g/in) and/or from about 118 g/cm (300 g/in) to about 1968 g/cm (5000 g/in) and/or from about 157 g/cm (400 g/in) to about 1181 g/cm (3000 g/in) and/or from about 196 g/cm (500 g/in) to about 984 g/cm (2500 g/in) and/or from about 196 g/cm (500 g/in) to about 787 g/cm (2000 g/in) and/or from about 196 g/cm (500 g/in) to about 591 g/cm (1500 g/in).

The sanitary tissue products of the present invention may exhibit a density of less than about 0.60 g/cm<sup>3</sup> and/or less than about 0.30 g/cm<sup>3</sup> and/or less than about 0.20 g/cm<sup>3</sup> and/or less than about 0.10 g/cm<sup>3</sup> and/or less than about 0.07 g/cm<sup>3</sup> and/or less than about 0.05 g/cm<sup>3</sup> and/or from about 0.01 g/cm<sup>3</sup> to about 0.20 g/cm<sup>3</sup> and/or from about 0.02 g/cm<sup>3</sup> to about 0.10 g/cm<sup>3</sup>.

The sanitary tissue products of the present invention may exhibit a total absorptive capacity of according to the Horizontal Full Sheet (HFS) Test Method described herein of greater than about 10 g/g and/or greater than about 12 g/g and/or greater than about 15 g/g and/or from about 15 g/g to about 50 g/g and/or to about 40 g/g and/or to about 30 g/g.

The sanitary tissue products of the present invention may exhibit a Vertical Full Sheet (VFS) value as determined by

the Vertical Full Sheet (VFS) Test Method described herein of greater than about 5 g/g and/or greater than about 7 µg and/or greater than about 9 g/g and/or from about 9 µg to about 30 µg and/or to about 25 g/g and/or to about 20 µg and/or to about 17 µg.

The sanitary tissue products of the present invention may be in the form of sanitary tissue product rolls. Such sanitary tissue product rolls may comprise a plurality of connected, but perforated sheets of fibrous structure, that are separably dispensable from adjacent sheets. In one example, one or more ends of the roll of sanitary tissue product may comprise an adhesive and/or dry strength agent to mitigate the loss of fibers, especially wood pulp fibers from the ends of the roll of sanitary tissue product.

The sanitary tissue products of the present invention may comprise additives such as softening agents, temporary wet strength agents, permanent wet strength agents, bulk softening agents, lotions, silicones, wetting agents, latexes, especially surface-pattern-applied latexes, dry strength agents such as carboxymethylcellulose and starch, and other types of additives suitable for inclusion in and/or on sanitary tissue products.

“Weight average molecular weight” as used herein means the weight average molecular weight as determined using gel permeation chromatography according to the protocol found in Colloids and Surfaces A. Physico Chemical & Engineering Aspects, Vol. 162, 2000, pg. 107-121.

“Basis Weight” as used herein is the weight per unit area of a sample reported in lbs/3000 ft<sup>2</sup> or g/m<sup>2</sup>.

“Machine Direction” or “MD” as used herein means the direction parallel to the flow of the fibrous structure through the fibrous structure making machine and/or sanitary tissue product manufacturing equipment.

“Cross Machine Direction” or “CD” as used herein means the direction parallel to the width of the fibrous structure making machine and/or sanitary tissue product manufacturing equipment and perpendicular to the machine direction.

“Ply” as used herein means an individual, integral fibrous structure.

“Plies” as used herein means two or more individual, integral fibrous structures disposed in a substantially contiguous, face-to-face relationship with one another, forming a multi-ply fibrous structure and/or multi-ply sanitary tissue product. It is also contemplated that an individual, integral fibrous structure can effectively form a multi-ply fibrous structure, for example, by being folded on itself.

“Total Pore Volume” as used herein means the sum of the fluid holding void volume in each pore range from 1 µm to 1000 µm radii as measured according to the Pore Volume Test Method described herein.

“Pore Volume Distribution” as used herein means the distribution of fluid holding void volume as a function of pore radius. The Pore Volume Distribution of a fibrous structure is measured according to the Pore Volume Test Method described herein.

Unless otherwise noted, the values of the properties of fibrous structures described herein are measured according to their corresponding Test Method, some of which are described herein.

As used herein, the articles “a” and “an” when used herein, for example, “an anionic surfactant” or “a fiber” is understood to mean one or more of the material that is claimed or described.

All percentages and ratios are calculated by weight unless otherwise indicated. All percentages and ratios are calculated based on the total composition unless otherwise indicated.

Unless otherwise noted, all component or composition levels are in reference to the active level of that component or composition, and are exclusive of impurities, for example, residual solvents or by-products, which may be present in commercially available sources.

#### Fibrous Structure

It has unexpectedly been found that the fibrous structures of the present invention exhibit improved absorbency and/or strength properties compared to known fibrous structures.

The fibrous structures of the present invention may comprise a plurality of filaments, a plurality of solid additives, such as fibers, and a mixture of filaments and solid additives.

The fibrous structures of the present invention that exhibit a VFS of greater than about 11 g/g may exhibit a pore volume distribution as exemplified in FIGS. 1 and 2, plots A and B. The fibrous structures of the present invention may exhibit a pore volume distribution such that greater than about 40% of the total pore volume present in the fibrous structure exists in pores of radii of from about 121  $\mu\text{m}$  to about 200  $\mu\text{m}$  and/or greater than about 50% of the total pore volume present in the fibrous structure exists in pores of radii of from about 101  $\mu\text{m}$  to about 200  $\mu\text{m}$ . The ranges of 101  $\mu\text{m}$  to 200  $\mu\text{m}$  and 121  $\mu\text{m}$  to 200  $\mu\text{m}$  are explicitly identified on the graph of FIG. 2. It should be noted that the value for the ending pore radius for the range of 101  $\mu\text{m}$  to 120  $\mu\text{m}$  is plotted at the ending pore radius; namely, 120  $\mu\text{m}$ . A similar result is shown on FIG. 2 for the value for the ending pore radius for the range of 121  $\mu\text{m}$  to 140  $\mu\text{m}$ , where the value is plotted at the ending pore radius; namely, 140  $\mu\text{m}$ . This data is also supported by the values present in Table 2 below.

The fibrous structures of the present invention have been found to exhibit consumer-recognizable beneficial absorbent capacity. In one example, the fibrous structures comprise a plurality of solid additives, for example fibers. In another example, the fibrous structures comprise a plurality of filaments. In yet another example, the fibrous structures comprise a mixture of filaments and solid additives, such as fibers.

As shown in FIG. 2, the examples of fibrous structures according to the present invention as represented by plots A and B may exhibit a bi-modal pore volume distribution such that the fibrous structure exhibits a pore volume distribution such that the greater than about 40% of the total pore volume present in the fibrous structure exists in pores of radii of from about 121  $\mu\text{m}$  to about 200  $\mu\text{m}$  and greater than about 2% and/or greater than about 5% and/or greater than about 10% of the total pore volume present in the fibrous structure exists in pores of radii of less than about 100  $\mu\text{m}$  and/or less than about 80  $\mu\text{m}$  and/or less than about 50  $\mu\text{m}$  and/or from about 1  $\mu\text{m}$  to about 100  $\mu\text{m}$  and/or from about 5  $\mu\text{m}$  to about 75  $\mu\text{m}$  and/or 10  $\mu\text{m}$  to about 50  $\mu\text{m}$ .

A fibrous structure according to the present invention exhibiting a bi-modal pore volume distribution as described above provides beneficial absorbent capacity and absorbent rate as a result of the larger radii pores and beneficial surface drying as a result of the smaller radii pores.

FIGS. 3 and 4 show schematic representations of an example of a fibrous structure in accordance with the present invention. As shown in FIGS. 3 and 4, the fibrous structure 10 may be a co-formed fibrous structure. The fibrous structure 10 comprises a plurality of filaments 12, such as polypropylene fibers, and a plurality of solid additives, such as wood pulp fibers 14. The filaments 12 may be randomly arranged as a result of the process by which they are spun and/or formed into the fibrous structure 10. The wood pulp fibers 14, may be randomly dispersed throughout the fibrous

structure 10 in the x-y plane. The wood pulp fibers 14 may be non-randomly dispersed throughout the fibrous structure in the z-direction. In one example (not shown), the wood pulp fibers 14 are present at a higher concentration on one or more of the exterior, x-y plane surfaces than within the fibrous structure along the z-direction.

As shown in FIG. 5, another example of a fibrous structure in accordance with the present invention is a layered fibrous structure 10'. The layered fibrous structure 10' comprises a first layer 16 comprising a plurality of filaments 12, such as polypropylene filaments, and a plurality of solid additives, in this example wood pulp fibers 14. The layered fibrous structure 10' further comprises a second layer 18 comprising a plurality of filaments 20, such as polypropylene filaments. In one example, the first and second layers 16, 18, respectively, are sharply defined zones of concentration of the filaments and/or solid additives. The plurality of filaments 20 may be deposited directly onto a surface of the first layer 16 to form a layered fibrous structure that comprises the first and second layers 16, 18, respectively.

Further, the layered fibrous structure 10' may comprise a third layer 22, as shown in FIG. 5. The third layer 22 may comprise a plurality of filaments 24, which may be the same or different from the filaments 20 in the second and/or first layers 18, 16. As a result of the addition of the third layer 22, the first layer 16 is positioned, for example sandwiched, between the second layer 18 and the third layer 22. The plurality of filaments 24 may be deposited directly onto a surface of the first layer 16, opposite from the second layer, to form the layered fibrous structure 10' that comprises the first, second and third layers 16, 18, 22, respectively.

As shown in FIG. 6, a cross-sectional schematic representation of another example of a fibrous structure in accordance with the present invention comprising a layered fibrous structure 10" is provided. The layered fibrous structure 10" comprises a first layer 26, a second layer 28 and optionally a third layer 30. The first layer 26 comprises a plurality of filaments 12, such as polypropylene filaments, and a plurality of solid additives, such as wood pulp fibers 14. The second layer 28 may comprise any suitable filaments, solid additives and/or polymeric films. In one example, the second layer 28 comprises a plurality of filaments 34. In one example, the filaments 34 comprise a polymer selected from the group consisting of: polysaccharides, polysaccharide derivatives, polyvinylalcohol, polyvinylalcohol derivatives and mixtures thereof.

In another example of a fibrous structure in accordance with the present invention, instead of being layers of fibrous structure 10", the material forming layers 26, 28 and 30, may be in the form of plies wherein two or more of the plies may be combined to form a fibrous structure. The plies may be bonded together, such as by thermal bonding and/or adhesive bonding, to form a multi-ply fibrous structure.

Another example of a fibrous structure of the present invention in accordance with the present invention is shown in FIG. 7. The fibrous structure 10''' may comprise two or more plies, wherein one ply 36 comprises any suitable fibrous structure in accordance with the present invention, for example fibrous structure 10 as shown and described in FIGS. 3 and 4 and another ply 38 comprising any suitable fibrous structure, for example a fibrous structure comprising filaments 40, such as polypropylene filaments. The fibrous structure of ply 38 may be in the form of a net and/or mesh and/or other structure that comprises pores that expose one or more portions of the fibrous structure 10 to an external environment and/or at least to liquids that may come into contact, at least initially, with the fibrous structure of ply 38.

In addition to ply 38, the fibrous structure 10<sup>'''</sup> may further comprise ply 42. Ply 42 may comprise a fibrous structure comprising filaments 44, such as polypropylene filaments, and may be the same or different from the fibrous structure of ply 38.

Two or more of the plies 36, 38 and 42 may be bonded together, such as by thermal bonding and/or adhesive bonding, to form a multi-ply fibrous structure. After a bonding operation, especially a thermal bonding operation, it may be difficult to distinguish the plies of the fibrous structure 10<sup>'''</sup> and the fibrous structure 10<sup>'''</sup> may visually and/or physically be a similar to a layered fibrous structure in that one would have difficulty separating the once individual plies from each other. In one example, ply 36 may comprise a fibrous structure that exhibits a basis weight of at least about 15 g/m<sup>2</sup> and/or at least about 20 g/m<sup>2</sup> and/or at least about 25 g/m and/or at least about 30 g/m<sup>2</sup> up to about 120 g/m<sup>2</sup> and/or 100 g/m<sup>2</sup> and/or 80 g/m<sup>2</sup> and/or 60 g/m<sup>2</sup> and the plies 38 and 42, when present, independently and individually, may comprise fibrous structures that exhibit basis weights of less than about 10 g/m<sup>2</sup> and/or less than about 7 g/m<sup>2</sup> and/or less than about 5 g/m<sup>2</sup> and/or less than about 3 g/m<sup>2</sup> and/or less than about 2 g/m<sup>2</sup> and/or to about 0 g/m<sup>2</sup> and/or 0.5 g/m<sup>2</sup>.

Plies 38 and 42, when present, may help retain the solid additives, in this case the wood pulp fibers 14, on and/or within the fibrous structure of ply 36 thus reducing lint and/or dust (as compared to a single-ply fibrous structure comprising the fibrous structure of ply 36 without the plies 38 and 42) resulting from the wood pulp fibers 14 becoming free from the fibrous structure of ply 36.

The fibrous structures of the present invention may comprise any suitable amount of filaments and any suitable amount of solid additives. For example, the fibrous structures may comprise from about 10% to about 70% and/or from about 20% to about 60% and/or from about 30% to about 50% by dry weight of the fibrous structure of filaments and from about 90% to about 30% and/or from about 80% to about 40% and/or from about 70% to about 50% by dry weight of the fibrous structure of solid additives, such as wood pulp fibers.

The filaments and solid additives of the present invention may be present in fibrous structures according to the present invention at weight ratios of filaments to solid additives of from at least about 1:1 and/or at least about 1:1.5 and/or at least about 1:2 and/or at least about 1:2.5 and/or at least about 1:3 and/or at least about 1:4 and/or at least about 1:5 and/or at least about 1:7 and/or at least about 1:10.

The fibrous structures of the present invention and/or any sanitary tissue products comprising such fibrous structures may be subjected to any post-processing operations such as embossing operations, printing operations, tuft-generating operations, thermal bonding operations, ultrasonic bonding operations, perforating operations, surface treatment operations such as application of lotions, silicones and/or other materials and mixtures thereof.

Any hydrophobic or non-hydrophilic materials within the fibrous structure, such as polypropylene filaments, may be surface treated and/or melt treated with a hydrophilic modifier. Nonlimiting examples of surface treating hydrophilic modifiers include surfactants, such as Triton X-100. Non-limiting examples of melt treating hydrophilic modifiers that are added to the melt, such as the polypropylene melt, prior to spinning filaments, include hydrophilic modifying melt additives such as VW351 commercially available from Polyvel, Inc. and Irgasurf commercially available from Ciba. The hydrophilic modifier may be associated with the

hydrophobic or non-hydrophilic material at any suitable level known in the art. In one example, the hydrophilic modifier is associated with the hydrophobic or non-hydrophilic material at a level of less than about 20% and/or less than about 15% and/or less than about 10% and/or less than about 5% and/or less than about 3% to about 0% by dry weight of the hydrophobic or non-hydrophilic material.

The fibrous structures of the present invention may include optional additives, each, when present, at individual levels of from about 0% and/or from about 0.01% and/or from about 0.1% and/or from about 1% and/or from about 2% to about 95% and/or to about 80% and/or to about 50% and/or to about 30% and/or to about 20% by dry weight of the fibrous structure. Nonlimiting examples of optional additives include permanent wet strength agents, temporary wet strength agents, dry strength agents such as carboxymethylcellulose and/or starch, softening agents, lint reducing agents, opacity increasing agents, wetting agents, odor absorbing agents, perfumes, temperature indicating agents, color agents, dyes, osmotic materials, microbial growth detection agents, antibacterial agents and mixtures thereof.

The fibrous structure of the present invention may itself be a sanitary tissue product. It may be convolutedly wound about a core to form a roll. It may be combined with one or more other fibrous structures as a ply to form a multi-ply sanitary tissue product. In one example, a co-formed fibrous structure of the present invention may be convolutedly wound about a core to form a roll of co-formed sanitary tissue product. The rolls of sanitary tissue products may also be coreless.

As shown in FIG. 8, a fibrous structure roll 46 comprising a fibrous structure, such as a fibrous structure according to the present invention, comprises end edges 48, 50. At least one of the end edges 48, 50 comprises a bond region 52. The bond region 52 may comprise a plurality of bond subregions (not shown) that are present at a frequency of at least about 10 and/or at least about 50 and/or at least about 100 and/or at least about 200 per inch, such as dots per inch (dpi). In one example, the bond region 52 may cover the entire or substantially the entire surface area of the end edge 48. In one example, the bond region 52 comprises greater than about 20% and/or greater than about 25% and/or greater than about 30% and/or greater than about 50% of the total surface area of the end edge 48. In one example, the bond region 52 is a film that comprises the entire or substantially entire total surface area of the end edge 48. In another example, the bond region 52 is present on a non-lotioned fibrous structure.

The bond region 52 may comprise a bonding agent selected from chemical agents and/or mechanical agents. Nonlimiting examples of chemical agents include dry strength agents and wet strength agents and mixtures thereof. The mechanical agents may be in the form of a liquid and/or a solid. A liquid mechanical agent may be an oil. A solid mechanical agent may be a wax.

The bond region 52 may comprise different types of bonding agents and/or bonding agents that are chemically different from the filaments and/or fibers present in the fibrous structure. In one example, the material comprises a bonding agent, such as a dry strength resin such as a polysaccharide and/or a polysaccharide derivative and temporary and permanent wet strength resins. Nonlimiting examples of suitable bonding agents include latex dispersions, polyvinyl alcohol, Parez<sup>®</sup>, Kymene<sup>®</sup>, carboxymethylcellulose and starch.

As shown in FIG. 9, a fibrous structure 54 in accordance with the present invention may comprise edges 56, 58, 60, 62. One or more of the edges 56, 58, 60, 62 may comprise a bond region 64. The bond region 64 may extend inwardly

## 11

from the edge 56, for example less than about 1 cm and/or less than about 0.5 cm. Any of the edges may comprise such a bond region. The bond region 64 may comprise a plurality of bond subregions (not shown) that are present at a frequency of at least 10 and/or at least 50 and/or at least 100 and/or at least 200 per inch, such as dots per inch (dpi). The bond region 64 may comprise a material chemically different from the filaments and/or fibers present in the fibrous structure. In one example, the material comprises a bonding agent, such as a dry strength resin such as a polysaccharide and/or a polysaccharide derivative. Nonlimiting examples of suitable bonding agents include carboxymethylcellulose and starch.

The fibrous structures of the present invention may exhibit a unique combination of fibrous structure properties that do not exist in known fibrous structures. For example, the fibrous structures may exhibit a VFS of greater than about 11 g/g and/or greater than about 12 g/g and/or greater than about 13 g/g and/or greater than about 14 g/g and/or less than about 50 g/g and/or less than about 40 g/g and/or less than about 30  $\mu$ g and/or less than about 20  $\mu$ g and/or from about 11 g/g to about 50  $\mu$ g and/or from about 11 g/g to about 40  $\mu$ g and/or from about 11 g/g to about 30 g/g and/or from about 11 g/g to about 20  $\mu$ g.

In addition to the VFS property, the fibrous structures of the present invention may exhibit a Dry CD Tensile Modulus of less than about 1500 g/cm and/or less than about 1400 g/cm and/or less than about 1300 g/cm and/or less than about 1100 g/cm and/or less than about 1000 g/cm and/or less than about 800 g/cm and/or greater than about 50 g/cm and/or greater than about 100 g/cm and/or greater than about 300 g/cm and/or from about 50 g/cm to about 1500 g/cm and/or from about 100 g/cm to about 1400 g/cm and/or from about 100 g/cm to about 1300 g/cm.

In addition to the VFS property and/or the Dry CD Tensile Modulus property, the fibrous structures of the present invention may exhibit a Wet CD TEA of greater than about

## 12

35 (g·in)/in<sup>2</sup> and/or greater than about 50 (g·in)/in<sup>2</sup> and/or greater than about 75 (g·in)/in<sup>2</sup> and/or greater than about 90 (g·in)/in<sup>2</sup> and/or greater than about 150 (g·in)/in<sup>2</sup> and/or greater than about 175 (g·in)/in<sup>2</sup> and/or less than about 500 (g·in)/in<sup>2</sup> and/or less than about 400 (g·in)/in<sup>2</sup> and/or less than about 350 (g·in)/in<sup>2</sup> and/or less than about 300 (g·in)/in<sup>2</sup> and/or from about 35 (g·in)/in<sup>2</sup> to about 500 (g·in)/in<sup>2</sup> and/or from about 35 (g·in)/in<sup>2</sup> to about 400 (g·in)/in<sup>2</sup> and/or from about 50 (g·in)/in<sup>2</sup> to about 350 (g·in)/in<sup>2</sup> and/or from about 75 (g·in)/in<sup>2</sup> to about 300 (g·in)/in<sup>2</sup>.

In addition to the VFS property and/or the Dry CD Tensile Modulus property and/or the Wet CD TEA, the fibrous structures of the present invention may exhibit a Wet MD TEA of greater than about 40 (g·in)/in<sup>2</sup> and/or greater than about 50 (g·in)/in<sup>2</sup> and/or greater than about 75 (g·in)/in<sup>2</sup> and/or greater than about 150 (g·in)/in<sup>2</sup> and/or greater than about 175 (g·in)/in<sup>2</sup> and/or less than about 500 (g·in)/in<sup>2</sup> and/or less than about 400 (g·in)/in<sup>2</sup> and/or less than about 350 (g·in)/in<sup>2</sup> and/or less than about 300 (g·in)/in<sup>2</sup> and/or from about 40 (g·in)/in<sup>2</sup> to about 500 (g·in)/in<sup>2</sup> and/or from about 35 (g·in)/in<sup>2</sup> to about 400 (g·in)/in<sup>2</sup> and/or from about 50 (g·in)/in<sup>2</sup> to about 350 (g·in)/in<sup>2</sup> and/or from about 75 (g·in)/in<sup>2</sup> to about 300 (g·in)/in<sup>2</sup>.

In one example of the fibrous structures of the present invention, the fibrous structure exhibits a VFS of greater than about 11 g/g and one or more of the following: a Dry CD Tensile Modulus of less than about 1500 g/cm and/or a Wet CD TEA of greater than about 35 (g·in)/in<sup>2</sup> and/or a Wet MD TEA of greater than about 40 (g·in)/in<sup>2</sup>.

The values of these properties associated with a fibrous structure are determined according to the respective test methods described herein.

To further illustrate the fibrous structures of the present invention, Table 1 sets forth certain properties of known and commercially available fibrous structures and a fibrous structure in accordance with the present invention.

TABLE 1

| Property                          | Duramax ® | Viva ® (Wetlaid) | Viva ® (Airlaid) | Bounty ® | Scott ® | Sparkle ® | Invention Example |
|-----------------------------------|-----------|------------------|------------------|----------|---------|-----------|-------------------|
| Wet MD TEA (g·in)/in <sup>2</sup> | 377       | 21.4             | 34.5             | 22.4     | 16.7    | 14.8      | 90                |
| Wet CD TEA (g·in)/in <sup>2</sup> | 340       | 22.6             | 31.7             | 18.1     | 8.9     | 8.1       | 209               |
| Dry CD Tensile Modulus g/cm       | 728       | 299              | 660              | 1844     | 1500    | 5900      | 400               |
| VFS g/g                           | 5.7       | 10.4             | 10.9             | 9.9      | 8       | 5.6       | 13                |

To further illustrate the fibrous structures of the present invention, Table 2 sets forth the average pore volume distributions of known and/or commercially available fibrous structures and a fibrous structure in accordance with the present invention.

TABLE 2

| Pore Radius ( $\mu$ m) | Huggies ® | Huggies ® Wash Cloth | Duramax | Concert EBT.055.1010 TBAL | LBAL-DUNI embossed | Bounty ® | Invention Example A | Invention Example B |
|------------------------|-----------|----------------------|---------|---------------------------|--------------------|----------|---------------------|---------------------|
| 1                      | 0         | 0                    | 0       | 0                         | 0                  | 0        | 0                   | 0                   |
| 2.5                    | 19.25     | 29.6                 | 32.4    | 33.65                     | 34.4               | 31.1     | 19.55               | 15.85               |
| 5                      | 11.65     | 16.1                 | 17.85   | 18.1                      | 18.25              | 17.6     | 12.4                | 7.95                |

TABLE 2-continued

| Pore Radius (μm) | Huggies ® Wash Cloth | Duramax | Concert EBT.055.1010 TBAL | LBAL-DUNI embossed | Invention Example A | Invention Example B |
|------------------|----------------------|---------|---------------------------|--------------------|---------------------|---------------------|
| 10               | 11.7                 | 12.6    | 28.5                      | 14.4               | 14.75               | 32.8                |
| 15               | 7.96                 | 7.05    | 101.7                     | 8.65               | 8.5                 | 52.3                |
| 20               | 7.15                 | 4.65    | 62.7                      | 6.45               | 6.4                 | 36.7                |
| 30               | 31.35                | 6.45    | 91.55                     | 9.1                | 9.55                | 54                  |
| 40               | 110.4                | 5.5     | 82.1                      | 26.3               | 127.25              | 47.8                |
| 50               | 133.05               | 6.5     | 77.35                     | 65.95              | 71.4                | 43.6                |
| 60               | 200.1                | 96.55   | 70.5                      | 74.7               | 59.95               | 38.9                |
| 70               | 302.45               | 144.85  | 61.65                     | 70.25              | 69.05               | 36.3                |
| 80               | 336.9                | 132.35  | 56.05                     | 102.05             | 95.05               | 33.9                |
| 90               | 250.9                | 150.8   | 49.3                      | 174.05             | 150.1               | 33                  |
| 100              | 160.15               | 162.8   | 48.3                      | 293                | 232.9               | 32.2                |
| 120              | 172.8                | 394.1   | 95.6                      | 693.4              | 464.15              | 64.7                |
| 140              | 85.1                 | 451.7   | 89.5                      | 162.55             | 176.45              | 68.5                |
| 160              | 54                   | 505.45  | 76.6                      | 19.35              | 49.6                | 74.8                |
| 180              | 37.3                 | 509.7   | 63.45                     | 10.15              | 24.3                | 78.5                |
| 200              | 30.15                | 450.95  | 50                        | 8.2                | 18.55               | 89.2                |
| 225              | 28.2                 | 409.15  | 51.6                      | 8.5                | 18.95               | 134.4               |
| 250              | 22.85                | 245.2   | 44                        | 7.5                | 16.25               | 149.8               |
| 275              | 22.15                | 144.1   | 40.25                     | 2.7                | 14.9                | 157.9               |
| 300              | 18.4                 | 101.3   | 35.95                     | 10.05              | 13.75               | 125.7               |
| 350              | 29.95                | 153.2   | 60.7                      | 10.9               | 25.4                | 145                 |
| 400              | 24.25                | 141.7   | 59.25                     | 9.65               | 26.65               | 52.4                |
| 500              | 45.6                 | 271.15  | 266.45                    | 15.75              | 116.85              | 56                  |
| 600              | 34.3                 | 230.95  | 291.9                     | 14.5               | 71.3                | 23.9                |
| 800              | 46.65                | 261.6   | 162.4                     | 24.3               | 34.25               | 34.9                |
| 1000             | 38.75                | 112.55  | 29.15                     | 24.9               | 30.35               | 24.9                |
| Total            | 2273.45              | 5158.6  | 2196.75                   | 1919.05            | 1999.25             | 1770.8              |
| 101-200 μm       | 16.7%                | 44.8%   | 17.1%                     | 46.6%              | 36.7%               | 21.2%               |
| 121-200 μm       | 9.1%                 | 37.2%   | 12.7%                     | 10.4%              | 13.5%               | 17.6%               |
|                  |                      |         |                           |                    |                     | 53.0%               |
|                  |                      |         |                           |                    |                     | 61.0%               |

## Process for Making a Fibrous Structure

A nonlimiting example of a process for making a fibrous structure according to the present invention is represented in FIG. 10. The process shown in FIG. 10 comprises the step of mixing a plurality of solid additives 14 with a plurality of filaments 12. In one example, the solid additives 14 are wood pulp fibers, such as SSK fibers and/or Eucalyptus fibers, and the filaments 12 are polypropylene filaments. The solid additives 14 may be combined with the filaments 12, such as by being delivered to a stream of filaments 12 from a hammermill 66 via a solid additive spreader 67 to form a mixture of filaments 12 and solid additives 14. The filaments 12 may be created by meltblowing from a meltblow die 68. The mixture of solid additives 14 and filaments 12 are collected on a collection device, such as a belt 70 to form a fibrous structure 72. The collection device may be a patterned and/or molded belt that results in the fibrous structure exhibiting a surface pattern, such as a non-random, repeating pattern. The molded belt may have a three-dimensional pattern on it that gets imparted to the fibrous structure 72 during the process.

In one example of the present invention, the fibrous structures are made using a die comprising at least one filament-forming hole, and/or 2 or more and/or 3 or more rows of filament-forming holes from which filaments are spun. At least one row of holes contains 2 or more and/or 3 or more and/or 10 or more filament-forming holes. In addition to the filament-forming holes, the die comprises fluid-releasing holes, such as gas-releasing holes, in one example air-releasing holes, that provide attenuation to the filaments formed from the filament-forming holes. One or more fluid-releasing holes may be associated with a fila-

35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
70

made by a die according to the present invention, as shown in FIG. 13. As is evidenced by FIG. 13, the fibrous structure made by a die according to the present invention may comprise filaments that exhibit an average filament diameter of less than 1  $\mu\text{m}$ . Such filaments are not seen in the fibrous structure made by the known knife-edge die as shown in FIG. 12.

After the fibrous structure 72 has been formed on the collection device, the fibrous structure 72 may be subjected to post-processing operations such as embossing, thermal bonding, tuft-generating operations, moisture-imparting operations, and surface treating operations to form a finished fibrous structure. One example of a surface treating operation that the fibrous structure may be subjected to is the surface application of an elastomeric binder, such as ethylene vinyl acetate (EVA), latexes, and other elastomeric binders. Such an elastomeric binder may aid in reducing the lint created from the fibrous structure during use by consumers. The elastomeric binder may be applied to one or more surfaces of the fibrous structure in a pattern, especially a non-random repeating pattern, or in a manner that covers or substantially covers the entire surface(s) of the fibrous structure.

In one example, the fibrous structure 72 and/or the finished fibrous structure may be combined with one or more other fibrous structures. For example, another fibrous structure, such as a filament-containing fibrous structure, such as a polypropylene filament fibrous structure may be associated with a surface of the fibrous structure 72 and/or the finished fibrous structure. The polypropylene filament fibrous structure may be formed by meltblowing polypropylene filaments (filaments that comprise a second polymer that may be the same or different from the polymer of the filaments in the fibrous structure 72) onto a surface of the fibrous structure 72 and/or finished fibrous structure. In another example, the polypropylene filament fibrous structure may be formed by meltblowing filaments comprising a second polymer that may be the same or different from the polymer of the filaments in the fibrous structure 72 onto a collection device to form the polypropylene filament fibrous structure. The polypropylene filament fibrous structure may then be combined with the fibrous structure 72 or the finished fibrous structure to make a two-ply fibrous structure—three-ply if the fibrous structure 72 or the finished fibrous structure is positioned between two plies of the polypropylene filament fibrous structure like that shown in FIG. 5 for example. The polypropylene filament fibrous structure may be thermally bonded to the fibrous structure 72 or the finished fibrous structure via a thermal bonding operation.

In yet another example, the fibrous structure 72 and/or finished fibrous structure may be combined with a filament-containing fibrous structure such that the filament-containing fibrous structure, such as a polysaccharide filament fibrous structure, such as a starch filament fibrous structure, is positioned between two fibrous structures 72 or two finished fibrous structures like that shown in FIG. 6 for example.

The process for making fibrous structure 72 may be close coupled (where the fibrous structure is convolutedly wound into a roll prior to proceeding to a converting operation) or directly coupled (where the fibrous structure is not convolutedly wound into a roll prior to proceeding to a converting operation) with a converting operation to emboss, print, deform, surface treat, or other post-forming operation known to those in the art. For purposes of the present invention, direct coupling means that the fibrous structure 72 can proceed directly into a converting operation rather than,

for example, being convolutedly wound into a roll and then unwound to proceed through a converting operation.

The process of the present invention may include preparing individual rolls of fibrous structure and/or sanitary tissue product comprising such fibrous structure(s) that are suitable for consumer use. The fibrous structure may be contacted by a bonding agent (such as an adhesive and/or dry strength agent), such that the ends of a roll of sanitary tissue product according to the present invention comprise such adhesive and/or dry strength agent.

The process may further comprise contacting an end edge of a roll of fibrous structure with a material that is chemically different from the filaments and fibers, to create bond regions that bond the fibers present at the end edge and reduce lint production during use. The material may be applied by any suitable process known in the art. Nonlimiting examples of suitable processes for applying the material include non-contact applications, such as spraying, and contact applications, such as gravure roll printing, extruding, surface transferring. In addition, the application of the material may occur by transfer from contact of a log saw and/or perforating blade containing the material since, for example, the perforating operation, an edge of the fibrous structure that may produce lint upon dispensing a fibrous structure sheet from an adjacent fibrous structure sheet may be created.

#### Nonlimiting Example of Process for Making a Fibrous Structure of the Present Invention:

A 47.5%:47.5%:5% blend of Exxon-Mobil PP3546 polypropylene: Sunoco CP20VM polypropylene: Polyvel S-1416 wetting agent is dry blended, to form a melt blend. The melt blend is heated to 475° F. through a melt extruder. A 10" wide Biax 12 row spinnerette with 192 nozzles per cross-direction inch, commercially available from Biax 35 Fiberfilm Corporation, is utilized. 32 nozzles per cross-direction inch of the 192 nozzles have a 0.018" inside diameter while the remaining nozzles are solid, i.e. there is no opening in the nozzle. Approximately 0.17 grams per hole per minute (ghm) of the melt blend is extruded from the 40 open nozzles to form meltblown filaments from the melt blend. Approximately 200 SCFM of compressed air is heated such that the air exhibits a temperature of 395° F. at the spinnerette. Approximately 175 grams/minute of Koch 4825 semi-treated SSK pulp is defibrillated through a hammermill to form SSK wood pulp fibers (solid additive). 330 SCFM of air at 85-90° F. and 85% relative humidity (RH) is drawn into the hammermill and carries the pulp fibers to a solid additive spreader. The solid additive spreader turns the pulp fibers and distributes the pulp fibers in the cross-direction such that the pulp fibers are injected into the meltblown filaments in a perpendicular fashion through a 2"×10" cross-direction (CD) slot. A forming box surrounds the area where the meltblown filaments and pulp fibers are commingled. This forming box is designed to reduce the 55 amount of air allowed to enter or escape from this commingling area; however, there is a 2"×12" opening in the bottom of the forming box designed to permit additional cooling air to enter. A forming vacuum pulls air through a forming fabric thus collecting the commingled meltblown filaments and pulp fibers to form a fibrous structure. The forming vacuum is adjusted until an additional 400 SCFM of room air is drawn into the slot in the forming box. The fibrous structure formed by this process comprises about 75% by dry fibrous structure weight of pulp and about 25% by dry 60 fibrous structure weight of meltblown filaments.

As shown in FIG. 14, the solid additive spreader 78 has an inlet 80 and an exit 82. Any suitable material known in

the art may be used to make the spreader 78. Nonlimiting examples of suitable materials include non-conductive materials. For example, stainless steel and/or sheet metal may be used to fabricate the spreader 78. A pulp and air mixture 84 created in the hammermill (not shown) enters the spreader 78 through a duct (not shown) connecting the hammermill and spreader 78 at greater than about 8,000 fpm velocity and/or greater than about 14,000 fpm. The inlet 80 is tilted at an angle  $\alpha$  at approximately 5° upstream from perpendicular of the exit 82. The exit 82 of the solid additive spreader 78 has a height H in the range of about 2.54 cm (1 inch) to about 25.40 cm (10 inches). The width W of the exit 82 is from about 1.27 cm (0.5 inch) to about 10.16 cm (4 inches). Typically the width W of the exit 82 is about 5.08 cm (2 inches). The length L of the spreader 78 is from about 60.96 cm (24 inches) to about 243.84 cm (96 inches) and/or from about 91.44 cm (36 inches) to about 182.88 cm (72 inches) and/or from about 121.92 cm (48 inches) to about 152.40 cm (60 inches). A tapering of the height H of the spreader 78 occurs from the inlet end 86 to the exit end 88 to continually accelerate the pulp and air mixture 84. This tapering is from about 10.16 cm (4 inches) in height at the inlet 80 to about 5.08 cm (2 inches) in height at the exit 82. However, the spreader 78 may incorporate other similar taperings. The inlet end 86 of the spreader 78 has a semi-circular arc from the top view with a radius of from about 7.62 cm (3 inches) to about 50.80 cm (20 inches) and/or from about 12.70 cm (5 inches) to about 25.40 cm (10 inches). As shown in FIG. 15, multiple semi-circular arcs can be assembled to produce the desired spreader width. Each semi-circular arc would comprise its own inlet 80 centered in each of these semi-circular arcs.

Optionally, a meltblown layer of the meltblown filaments can be added to one or both sides of the above formed fibrous structure. This addition of the meltblown layer can help reduce the lint created from the fibrous structure during use by consumers and is preferably performed prior to any thermal bonding operation of the fibrous structure. The meltblown filaments for the exterior layers can be the same or different than the meltblown filaments used on the opposite layer or in the center layer(s).

The fibrous structure may be convolutedly wound to form a roll of fibrous structure. The end edges of the roll of fibrous structure may be contacted with a material to create bond regions.

#### Test Methods

Unless otherwise indicated, all tests described herein including those described under the Definitions section and the following test methods are conducted on samples that have been conditioned in a conditioned room at a temperature of 73° F. $\pm$ 4° F. (about 23° C. $\pm$ 2.2° C.) and a relative humidity of 50% $\pm$ 10% for 2 hours prior to the test. Samples conditioned as described herein are considered dry samples (such as "dry fibrous structures") for purposes of this invention. Further, all tests are conducted in such conditioned room.

#### A. Pore Volume Distribution Test Method

Pore Volume Distribution measurements are made on a TRI/Autoporosimeter (TRI/Princeton Inc. of Princeton, N.J.). The TRI/Autoporosimeter is an automated computer-controlled instrument for measuring pore volume distributions in porous materials (e.g., the volumes of different size pores within the range from 1 to 1000  $\mu$ m effective pore radii). Complimentary Automated Instrument Software, Release 2000.1, and Data Treatment Software, Release 2000.1 is used to capture, analyze and output the data. More information on the TRI/Autoporosimeter, its operation and

data treatments can be found in The Journal of Colloid and Interface Science 162 (1994), pgs 163-170, incorporated here by reference.

As used in this application, determining Pore Volume Distribution involves recording the increment of liquid that enters a porous material as the surrounding air pressure changes. A sample in the test chamber is exposed to precisely controlled changes in air pressure. The size (radius) of the largest pore able to hold liquid is a function of the air pressure. As the air pressure increases (decreases), different size pore groups drain (absorb) liquid. The pore volume of each group is equal to this amount of liquid, as measured by the instrument at the corresponding pressure. The effective radius of a pore is related to the pressure differential by the following relationship.

$$\text{Pressure differential} = [(2)\gamma \cos \Theta]/\text{effective radius}$$

where  $\gamma$ =liquid surface tension, and  $\Theta$ =contact angle.

Typically pores are thought of in terms such as voids, holes or conduits in a porous material. It is important to note that this method uses the above equation to calculate effective pore radii based on the constants and equipment controlled pressures. The above equation assumes uniform cylindrical pores. Usually, the pores in natural and manufactured porous materials are not perfectly cylindrical, nor all uniform. Therefore, the effective radii reported here may not equate exactly to measurements of void dimensions obtained by other methods such as microscopy. However, these measurements do provide an accepted means to characterize relative differences in void structure between materials.

The equipment operates by changing the test chamber air pressure in user-specified increments, either by decreasing pressure (increasing pore size) to absorb liquid, or increasing pressure (decreasing pore size) to drain liquid. The liquid volume absorbed (drained) at each pressure increment is the cumulative volume for the group of all pores between the preceding pressure setting and the current setting.

In this application of the TRI/Autoporosimeter, the liquid is a 0.2 weight % solution of octylphenoxy polyethoxy ethanol (Triton X-100 from Union Carbide Chemical and Plastics Co. of Danbury, Conn.) in distilled water. The instrument calculation constants are as follows:  $\rho$  (density) = 1 g/cm<sup>3</sup>;  $\gamma$  (surface tension)=31 dynes/cm;  $\cos \Theta$ =1. A 0.22  $\mu$ m Millipore Glass Filter (Millipore Corporation of Bedford, Mass.; Catalog #GSPW09025) is employed on the test chamber's porous plate. A plexiglass plate weighing about 24 g (supplied with the instrument) is placed on the sample to ensure the sample rests flat on the Millipore Filter. No additional weight is placed on the sample.

The remaining user specified inputs are described below. The sequence of pore sizes (pressures) for this application is as follows (effective pore radius in  $\mu$ m): 1, 2.5, 5, 10, 15, 20, 30, 40, 50, 60, 70, 80, 90, 100, 120, 140, 160, 180, 200, 225, 250, 275, 300, 350, 400, 500, 600, 800, 1000. This sequence starts with the sample dry, saturates it as the pore settings increase (typically referred to with respect to the procedure and instrument as the 1<sup>st</sup> absorption).

In addition to the test materials, a blank condition (no sample between plexiglass plate and Millipore Filter) is run to account for any surface and/or edge effects within the chamber. Any pore volume measured for this blank run is subtracted from the applicable pore grouping of the test sample. This data treatment can be accomplished manually or with the available TRI/Autoporosimeter Data Treatment Software, Release 2000.1.

Percent (%) Total Pore Volume is a percentage calculated by taking the volume of fluid in the specific pore radii range divided by the Total Pore Volume. The TRI/Autoporosimeter outputs the volume of fluid within a range of pore radii. The first data obtained is for the "2.5 micron" pore radii which includes fluid absorbed between the pore sizes of 1 to 2.5 micron radius. The next data obtained is for "5 micron" pore radii, which includes fluid absorbed between the 2.5 micron and 5 micron radii, and so on. Following this logic, to obtain the volume held within the range of 101-200 micron radii, one would sum the volumes obtained in the range titled "120 micron", "140 micron", "160 micron", "180 micron", and finally the "200 micron" pore radii ranges. For example, % Total Pore Volume 101-200 micron pore radii=(volume of fluid between 101-200 micron pore radii)/Total Pore Volume

B. Horizontal Full Sheet (HFS) Test Method

The Horizontal Full Sheet (HFS) test method determines the amount of distilled water absorbed and retained by a fibrous structure of the present invention. This method is performed by first weighing a sample of the fibrous structure to be tested (referred to herein as the "dry weight of the sample"), then thoroughly wetting the sample, draining the wetted sample in a horizontal position and then reweighing (referred to herein as "wet weight of the sample"). The absorptive capacity of the sample is then computed as the amount of water retained in units of grams of water absorbed by the sample. When evaluating different fibrous structure samples, the same size of fibrous structure is used for all samples tested.

The apparatus for determining the HFS capacity of fibrous structures comprises the following:

1) An electronic balance with a sensitivity of at least  $\pm 0.01$  grams and a minimum capacity of 1200 grams. The balance should be positioned on a balance table and slab to minimize the vibration effects of floor/benchtop weighing. The balance should also have a special balance pan to be able to handle the size of the sample tested (i.e.; a fibrous structure sample of about 11 in. (27.9 cm) by 11 in. (27.9 cm)). The balance pan can be made out of a variety of materials. Plexiglass is a common material used.

2) A sample support rack (FIG. 16) and sample support rack cover (FIG. 17) is also required. Both the rack and cover are comprised of a lightweight metal frame, strung with 0.012 in. (0.305 cm) diameter monofilament so as to form a grid as shown in FIG. 16. The size of the Support rack and cover is such that the sample size can be conveniently placed between the two.

The HFS test is performed in an environment maintained at  $23\pm 1^\circ$  C. and  $50\pm 2\%$  relative humidity. A water reservoir or tub is filled with distilled water at  $23\pm 1^\circ$  C. to a depth of 3 inches (7.6 cm).

Eight samples of a fibrous structure to be tested are carefully weighed on the balance to the nearest 0.01 grams. The dry weight of each sample is reported to the nearest 0.01 grams. The empty sample support rack is placed on the balance with the special balance pan described above. The balance is then zeroed (tared). One sample is carefully placed on the sample support rack. The support rack cover is placed on top of the support rack. The sample (now sandwiched between the rack and cover) is submerged in the water reservoir. After the sample is submerged for 60 seconds, the sample support rack and cover are gently raised out of the reservoir.

The sample, support rack and cover are allowed to drain horizontally for  $120\pm 5$  seconds, taking care not to excessively shake or vibrate the sample. While the sample is draining, the rack cover is carefully removed and all excess

water is wiped from the support rack. The wet sample and the support rack are weighed on the previously tared balance. The weight is recorded to the nearest 0.01 g. This is the wet weight of the sample.

5 The gram per fibrous structure sample absorptive capacity of the sample is defined as (wet weight of the sample-dry weight of the sample). The horizontal absorbent capacity (HAC) is defined as: absorvent capacity=(wet weight of the sample-dry weight of the sample)/(dry weight of the sample) and has a unit of gram/gram.

10 C. Vertical Full Sheet (VFS) Test Method

The Vertical Full Sheet (VFS) test method determines the amount of distilled water absorbed and retained by a fibrous structure of the present invention. This method is performed by first weighing a sample of the fibrous structure to be tested (referred to herein as the "dry weight of the sample"), then thoroughly wetting the sample, draining the wetted sample in a vertical position and then reweighing (referred to herein as "wet weight of the sample"). The absorptive 15 capacity of the sample is then computed as the amount of water retained in units of grams of water absorbed by the sample. When evaluating different fibrous structure samples, the same size of fibrous structure is used for all samples tested.

20 25 The apparatus for determining the VFS capacity of fibrous structures comprises the following:

1) An electronic balance with a sensitivity of at least  $\pm 0.01$  grams and a minimum capacity of 1200 grams. The balance should be positioned on a balance table and slab to 30 minimize the vibration effects of floor/benchtop weighing. The balance should also have a special balance pan to be able to handle the size of the sample tested (i.e.; a fibrous structure sample of about 11 in. (27.9 cm) by 11 in. (27.9 cm)). The balance pan can be made out of a variety of materials. Plexiglass is a common material used.

2) A sample support rack (FIG. 16) and sample support 35 rack cover (FIG. 17) is also required. Both the rack and cover are comprised of a lightweight metal frame, strung with 0.012 in. (0.305 cm) diameter monofilament so as to 40 form a grid as shown in FIG. 16. The size of the support rack and cover is such that the sample size can be conveniently placed between the two.

The VFS test is performed in an environment maintained at  $23\pm 1^\circ$  C. and  $50\pm 2\%$  relative humidity. A water reservoir or tub is filled with distilled water at  $23\pm 1^\circ$  C. to a depth of 45 3 inches (7.6 cm).

Eight 19.05 cm (7.5 inch)  $\times$  19.05 cm (7.5 inch) to 27.94 cm (11 inch)  $\times$  27.94 cm (11 inch) samples of a fibrous structure to be tested are carefully weighed on the balance to the nearest 0.01 grams. The dry weight of each sample is reported to the nearest 0.01 grams. The empty sample support rack is placed on the balance with the special balance pan described above. The balance is then zeroed (tared). One sample is carefully placed on the sample 50 support rack. The support rack cover is placed on top of the support rack. The sample (now sandwiched between the rack and cover) is submerged in the water reservoir. After the sample is submerged for 60 seconds, the sample support rack and cover are gently raised out of the reservoir.

55 60 The sample, support rack and cover are allowed to drain vertically for  $60\pm 5$  seconds, taking care not to excessively shake or vibrate the sample. While the sample is draining, the rack cover is carefully removed and all excess water is wiped from the support rack. The wet sample and the support rack are weighed on the previously tared balance. The weight is recorded to the nearest 0.01 g. This is the wet 65 weight of the sample.

The procedure is repeated for with another sample of the fibrous structure, however, the sample is positioned on the support rack such that the sample is rotated 90° compared to the position of the first sample on the support rack.

The gram per fibrous structure sample absorptive capacity of the sample is defined as (wet weight of the sample–dry weight of the sample). The calculated VFS is the average of the absorptive capacities of the two samples of the fibrous structure.

D. Wet MD TEA, Wet CD TEA, Dry CD Tensile Modulus (“Tangent Modulus”) Test Methods

The Wet MD TEA, Wet CD TEA and Dry CD Tensile Modulus of a fibrous structure are all determined using a Thwing Albert EJA Tensile Tester. A 2.54 cm (1 inch) wide strip of the fibrous structure to be tested is placed in the grips of the Tensile Tester at a gauge length of 10.16 cm (4 inches). The Crosshead Speed of the Tensile Tester is set at 10.16 cm/min (4 inches/min) and the Break Sensitivity is set at 20 g. Eight (8) samples are run on the Tensile Tester and an average of the respective Wet MD TEA, Wet CD TEA values from the 8 samples is reported as the Wet MD TEA value and the Wet CD TEA. The Dry CD Tensile Modulus is reported as the average of the Dry CD Tensile Modulus from the 8 samples measured at 15 g/cm.

E. Basis Weight Test Method

Basis weight is measured by preparing one or more samples of a certain area (m<sup>2</sup>) and weighing the sample(s) of a fibrous structure according to the present invention and/or a paper product comprising such fibrous structure on a top loading balance with a minimum resolution of 0.01 g. The balance is protected from air drafts and other disturbances using a draft shield. Weights are recorded when the readings on the balance become constant. The average weight (g) is calculated and the average area of the samples (m<sup>2</sup>). The basis weight (g/m<sup>2</sup>) is calculated by dividing the average weight (g) by the average area of the samples (m<sup>2</sup>).

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as “40 mm” is intended to mean “about 40 mm.”

All documents cited in the Detailed Description of the Invention are, in relevant part, incorporated herein by reference; the citation of any document is not to be construed as an admission that it is prior art with respect to the present invention. To the extent that any meaning or definition of a term in this document conflicts with any meaning or definition of the same term in a document incorporated by reference, the meaning or definition assigned to that term in this document shall govern.

While particular embodiments of the present invention have been illustrated and described, it would be obvious to those skilled in the art that various other changes and modifications can be made without departing from the spirit and scope of the invention. It is therefore intended to cover in the appended claims all such changes and modifications that are within the scope of this invention.

What is claimed is:

1. A multi-ply absorbent towel product in roll form comprising a plurality of perforated sheets, wherein the multi-ply absorbent towel product comprises a co-formed fibrous structure comprising a plurality of filaments, wherein the filaments comprise an internal wetting agent and wherein at least one of the filaments exhibits a length of 5.08 cm or greater and a plurality of solid additives randomly dispersed

throughout the co-formed fibrous structure wherein at least one of the solid additives comprises a fiber, wherein the multi-ply absorbent towel product exhibits a pore volume distribution such that greater than 60% of the total pore volume present in the multi-ply absorbent towel product exists in pores of radii of greater than 121 µm, and wherein the multi-ply absorbent towel product exhibits a VFS of greater than about 11 g/g, a basis weight of from about 10 g/m<sup>2</sup> to about 120 g/m<sup>2</sup>, and a density of less than 0.60 g/cm<sup>3</sup>.

2. The multi-ply absorbent towel product according to claim 1 wherein the fiber comprises a wood pulp fiber.

3. The multi-ply absorbent towel product according to claim 2 wherein the wood pulp fiber is selected from the group consisting of: Southern Softwood Kraft pulp fibers, Northern Softwood Kraft pulp fibers, Eucalyptus pulp fibers, Acacia pulp fibers.

4. The multi-ply absorbent towel product according to claim 1 wherein at least one of the plurality of filaments comprises a thermoplastic polymer.

5. The multi-ply absorbent towel product according to claim 4 wherein the thermoplastic polymer is selected from the group consisting of: polypropylene, polyethylene, polyester, polylactic acid, polyhydroxyalkanoate, polycaprolactone and mixtures thereof.

6. The multi-ply absorbent towel product according to claim 1 wherein at least one of the plurality of filaments comprises a natural polymer.

7. The multi-ply absorbent towel product according to claim 6 wherein the natural polymer is selected from the group consisting of: starch, starch derivatives, cellulose, cellulose derivatives, hemicellulose, hemicellulose derivatives and mixtures thereof.

8. The multi-ply absorbent towel product according to claim 1 wherein at least one surface of the multi-ply absorbent towel product comprises a layer of the filaments.

9. The multi-ply absorbent towel product according to claim 1 wherein the multi-ply absorbent towel product further exhibits one or more of the following properties: a Dry CD Tensile Modulus of less than about 1500 g/cm and/or a Wet CD TEA of greater than about 35 (g·in)/in<sup>2</sup> and/or a Wet MD TEA of greater than about 40 (g·in)/in<sup>2</sup>.

10. An osmotic material-free multi-ply absorbent towel product in roll form comprising a plurality of perforated sheets, wherein the multi-ply absorbent towel product comprises a co-formed fibrous structure comprising a plurality of filaments, wherein the filaments comprise an internal wetting agent and wherein at least one of the filaments exhibits a length of 5.08 cm or greater and a plurality of solid additives randomly dispersed throughout the co-formed fibrous structure wherein at least one of the solid additives comprises a fiber, wherein the multi-ply absorbent towel product exhibits a pore volume distribution such that greater than 60% of the total pore volume present in the multi-ply absorbent towel product exists in pores of radii of greater than 121 µm, and wherein the multi-ply absorbent towel product exhibits a VFS of greater than about 11 g/g, and wherein the multi-ply absorbent towel product further exhibits a basis weight of from about 10 g/m<sup>2</sup> to about 120 g/m<sup>2</sup> and a density of less than 0.60 g/cm<sup>3</sup>.

11. The multi-ply absorbent towel product according to claim 10 wherein the multi-ply absorbent towel product further exhibits one or more of the following properties: a Dry CD Tensile Modulus of less than about 1500 g/cm

and/or a Wet CD TEA of greater than about 35 (g·in)/in<sup>2</sup>  
and/or a Wet MD TEA of greater than about 40 (g·in)/in<sup>2</sup>.

\* \* \* \* \*